

June 6, 1939.

J. KIPPERMAN ET AL

2,161,419

METHOD OF MANUFACTURING CONDENSER ELECTRODES

Filed Aug. 21, 1936

Fig. 2



Fig. 1



Fig. 4



Fig. 5

INVENTORS  
JAN KIPPERMAN AND  
ADRIAAN JAN JURIAAN LAMBEK  
BY *H.S. Brown*  
ATTORNEY

## UNITED STATES PATENT OFFICE

2,161,419

## METHOD OF MANUFACTURING CONDENSER ELECTRODES

Jan Kipperman and Adriaan Jan Juriaan Lambeek, Tilburg, Netherlands, assignors to N. V. Philips' Gloeilampenfabrieken, Eindhoven, Netherlands

Application August 21, 1936, Serial No. 97,200  
In Germany September 2, 1935

6 Claims. (Cl. 29—155.5)

The invention relates to a method of manufacturing condenser electrodes built up from a plurality of concentric rings of substantially the same height and with equal wall thicknesses and intervening spaces which rings are arranged on a common bottom. Condenser electrodes of this kind are known already. The known electrodes are manufactured by concentrically securing, for example by soldering, a plurality of rings to a common bottom, so as to be mutually concentric. It has also previously been proposed to manufacture the electrodes by arranging a plurality of cup-shaped bodies so as to be mutually concentric and to secure the bottoms thereof to one another. The condenser is built up from two of such electrodes capable of being slid into one another.

The invention consists in manufacturing the whole of the electrode from a single piece of material in a single operation with the aid of the "cold squirting process" which is known per se.

The cold squirting process is utilised, for example, in the manufacture of cup-shaped bodies from a single piece of material, e. g., aluminium, the material being pressed through a single slit (die).

However, the manufacture of bodies of more complicated shape in which the material is simultaneously pressed through a plurality of slits, is beset, as is well-known, with drawbacks which consist in that the desired deformation is restricted to determined zones and is brought about at other points only imperfectly or not at all. This phenomenon is probably due to the fact that the material preferably flows towards the zones with the slightest resistances against deformation or frictional resistances. For this reason the cold-squirting process has hitherto remained restricted to bodies of simple shape. According to the invention, by taking particular measures it becomes possible to produce in this way also bodies of very complicated shape.

The starting-point is formed by the following considerations: On considering the article before and after deformation, one would expect the afflux or cold flow of the material of each ring from that region of the material which has not yet been brought into its final shape, which is located in the immediate vicinity of the ring in question. If, as indicated in Fig. 3, the distances between the rings are divided into two, it would be obvious that, when considering the zones between these lines of separation to be zones of afflux of the enclosed rings, with these apparent zones of afflux an equal height for all rings could be obtained if

the width b of the zones of afflux would be equal for all rings.

When deforming in accordance with said obvious idea, it is found that the inner rings are formed only very imperfectly and the product obtained is unfit for practical use. It appears therefrom that the resistance against deformation strongly increases towards the middle. The applicants have gained the recognition that the zone of afflux which really occurs differs from the above-mentioned apparent zone of afflux. The real zone of afflux of a ring is to be understood to mean the region from which originates the material of the ring under consideration.

On the ground of this recognition the applicants have found that by giving the tool to be employed the correct shape the form of the real zones of afflux can be acted upon in such manner that the final shape of the body to be produced can be determined beforehand.

According to the invention, the apparent zone of afflux of the outermost ring is reduced. It has been found that in this way the real zones of afflux of all rings, from the inside to the outside, are reduced more and more.

As mentioned above, the resistance against deformation increases from the outside to the inside and the rings located further outwards take a larger height.

When taking the measure according to the invention the real zones of afflux of the different rings are acted upon in such manner that the inward increase of the resistance, against deformation, which results in the unequal height of the rings, is neutralized and that bodies as those above described may be manufactured from a single piece of material according to the cold-squirting method.

The invention will be explained more fully with reference to the accompanying drawing. Although for the sake of simplicity only a slight number of rings is shown, it is clear that in accordance with the invention electrodes may be manufactured which consist of any desired number of rings.

Fig. 1 represents a condenser electrode consisting of a bottom 1 and of rings 2, 3 and 4. The bottom is provided at the outside with a flange 5. It would be possible to turn such a body. According to the invention such a body is produced with the aid of the cold-squirting process. As previously mentioned, this method is known for squirting bodies of simple, e. g. cup-shaped form. Use is made in that case of a device consisting of two parts. Building further on that

which is known, one arrives at the device shown in Fig. 2 which consists of a stationary table 6 and a movable stamp or die. A pastil or metal blank P is placed on the table. The stamp comprises a body pierced with a cylindrical aperture and a plurality of annular stamp portions 9 and 10. The body 7 has a widened portion 11 in which the flange is formed which is required for the easy removal of the body after the moulding operation. The applicants have found, however that such a mould would be completely unfit for use because there would be produced an electrode as shown in Fig. 3.

It is impossible to mould with this device in such manner that the inner rings, too, acquire a sufficient height. The applicants have found that this phenomenon has to be ascribed to the causes mentioned hereafter.

Fig. 3 shows diagrammatically the apparent zones of afflux. The apparent zone of afflux 12 of the outermost ring is substantially equal to the apparent zones of afflux 13 and 14 of the rings located more inwards. It has been found, however, that with this mould the real zone of afflux 25 of the outer rings is much larger than that of the inner rings and that the extension of the real zones of afflux decreases inwardly. This phenomenon results from the greater resistance against deformation experienced by the material in the neighbourhood of the rings located farther inwardly. According to the invention, this drawback may be removed by reducing the apparent zone of afflux of the outermost ring. It has been found that this measure acts upon the real zones 35 of afflux of all rings in such manner that for each ring which is located more outwardly less material is available, owing to which all rings acquire a substantially equal height. This may be ensured, for example, by suppressing the annular 40 cavity 11 in Fig. 2 which, on shallow consideration, would be required in order to obtain the desired shape. There is produced in this case a condenser electrode according to Fig. 4 which is smooth on the outside and whose rings have substantially the same height. It will be seen that the apparent zone of afflux 15 of the outermost ring is smaller than the apparent zones of afflux 16 of the following rings. The apparent zones of afflux of the other rings are equal. There is produced in this way a central aperture with a narrowed portion which may be utilized, if desired, for the expulsion of the work-piece.

As results from the above, a radial displacement of the material during deformation is required in order to obtain the desired deformation. It is necessary for this purpose that in the achieved electrode the thickness of the bottom is large relatively to the thickness of the rings, for example four times as large. Slight disparities in the height of the rings may be compensated for in the manner usually applied in technics.

An electrode according to the invention having the flange 5 shown in Fig. 1 may be manufactured with the aid of the moulding device represented in Fig. 5. This device consists of a table 17 and of a body 18 arranged thereon which does not move together with the stamp and which has an annular recess 19. P denotes again the pastil. The stamp has a pin 20 and a few annular stamp portions 21, 22 and 23. It has been found that with this mould, too, the apparent zone of afflux of the outermost ring is smaller than those of the other rings so that the desired effect is ensured. The lower surface of the bottom of the

electrode may have any desired profile which is simultaneously pressed into it.

The applicants have found that the increase of the zone of afflux for the innermost ring, which may be obtained, for example, by suppressing or reducing the aperture in the bottom, acts almost exclusively on the deformation of the inner rings but does not extend to the rings located further outwards. A central aperture is consequently always indispensable. This does, however, not entail any disadvantage, for this aperture may serve very well for the attachment of the electrode in the condenser. This is particularly important with adjustable condensers. Through said aperture may be passed in this case, for example, a spindle on which the electrode is slideable.

The electrode according to the invention affords, in addition to its cheap manufacture, the further advantage that the distance between two 20 rings is always the same. Besides, all electrodes manufactured with one and the same device, are exactly identical so that the disparities in the values of the capacities of different condensers may be kept very small.

As the material may be utilised first of all aluminium and then also brass with a sufficient content of copper, lead and zinc. In general any material utilised in cold-squirtting may be employed. A previous heating of the pastil may be 30 advantageous. If use is made of aluminium, the heating temperature should preferably amount to about 200° C.

What we claim is:

1. The method of making a condenser electrode having a smooth outside wall and a plurality of rings of substantially the same height from a single piece of metal by cold squirming process which comprises placing a circular blank of metal on a stationary table and confining said blank within a circular body arranged on said stationary table, forming said blank of metal by applying pressure on a movable die having a central guide pin, and a plurality of annular rings, the arrangement of each ring being such that the real zones of afflux of all of the rings from the inside to the outside are reduced more and more to provide equal height of the rings thus formed.

2. The method of making a condenser electrode from a single piece of metal by cold squirming process which comprises heating a blank of aluminum metal to approximately two hundred degrees centigrade, placing said aluminum blank on a stationary table, and confining said aluminum blank within a circular body arranged on said stationary table, forming said blank of aluminum by applying pressure on a movable die having a central guide pin, and a plurality of annular rings, the arrangement of each ring being such that the real zones of afflux of all the rings from the inside to the outside are reduced more and more to provide equal height of the rings thus formed.

3. The method of making a condenser electrode from a single piece of metal by cold squirming process which comprises placing a circular blank of metal on a stationary table and confining said blank within a circular body arranged on said stationary table, forming said blank of metal by applying pressure on a movable die having a central guide pin, and a plurality of annular rings, the arrangement of each ring being such that the apparent zone of afflux of the metal of the outer ring is reduced so that the real

zones of afflux of all the rings from the inside to the outside are reduced more and more to provide equal height of the rings thus formed.

4. The method of making a condenser electrode having a thickness which is large at the bottom relative to the thickness of a plurality of rings, from a single piece of metal by cold squirming process which comprises placing a circular blank of metal on a stationary table and confining said blank within a circular body arranged on said stationary table, forming said blank of metal by applying pressure on a movable die having a central guide pin, and a plurality of annular rings, the arrangement of each ring being such that the real zones of afflux of all the rings from the inside to the outside are reduced more and more to provide equal height of the rings thus formed.

5. The method of making a condenser electrode having its thickness at least four times as large at the bottom relative to the thickness of a plurality of rings, from a single piece of metal, by cold squirming process which comprises placing a circular blank of metal on a stationary table and confining said blank within a circular body

arranged on said stationary table, forming said blank of metal by applying pressure on a movable die having a central guide pin, and a plurality of annular rings, the arrangement of each ring being such that the real zones of afflux of all the rings from the inside to the outside are reduced more and more to provide equal height of the rings thus formed. 5

6. The method of making a condenser electrode from a single piece of metal by cold squirming process which comprises placing a circular blank of metal having a central aperture on a stationary table and confining said blank within a circular body arranged on said stationary table, forming said blank of metal by applying pressure 10 on a movable die having a central guide pin, and a plurality of annular rings, the arrangement of each ring being such that the real zones of afflux of all the rings from the inside to the outside are reduced more and more to provide equal 15 height of the rings thus formed, the central guide pin passing through the aperture in said guide. 20

JAN KIPPERMAN.

ADRIAAN JAN JURIAAN LAMBEEK. 25